# EUROPEAN PATENT SPECIFICATION

(11) **EP 2 216 433 B1**
(45) Date of publication and mention of the grant of the patent: **03.02.2016**
(21) Application number: 10152917.0
(22) Date of filing: 08.02.2010
(51) Int. Cl.: D03D 1/00, D03D 11/02, D03D 15/12, E06B 9/262, E06B 9/266, E06B 9/38

(54) **3-D fabric and preparing thereof**
3-D-Stoff und Herstellung davon
Tissu 3D et sa préparation

(30) Priority: 09.02.2009 KR 20090009997
(43) Date of publication of application: 11.08.2010
(73) Proprietor: Youil Corporation Co., Ltd., Gyeongsangbuk-do 719-853 (KR)
(72) Inventor: Chang, Hoo-Sung, Seoul 134-060 (KR); Ryu, Il-Sun, Nam-gu Daegu 705-752 (KR)
(74) Representative: Grünecker Patent- und Rechtsanwälte PartG mbB

(56) References cited:
- EP-A1- 0 447 058
- EP-A2- 0 733 730
- WO-A1-2008/127030
- FR-A1- 2 907 475
- GB-A- 722 090

## Description

### [Technical Field]

The present invention relates to fabrics that can create three-dimensional shapes and methods for the production of the fabrics. More specifically, the present invention relates to fabrics, particularly fabrics applicable as materials for blinds with high light-shielding rate due to intermediate portions having a multi-layered structure, that can be woven on a single loom in a batch operation by novel weaving techniques and undergo transformation between two-dimensional and three-dimensional shapes, and methods for the production of the fabrics.

### [Background Art]

Fabrics are typically made from corresponding raw materials and are constructed by weaving, knitting, plaiting or braiding. For example, felt fabrics are produced by the interlocking of fibers. Fabrics are primarily classified into woven fabrics, knitted fabrics, felt fabrics, plaited fabrics, non-woven fabrics, laminated fabrics and molded fabrics by standard production methods thereof.

In a narrow sense, woven fabrics refer to fabrics constructed by interlacing vertical warp threads with horizontal weft threads at right angles. Woven fabrics are the most widely used fabrics for under wears and outer wears. Knitted fabrics are constructed by making sets of threads into loops and combining the loops with one another in forward, backward, left and right directions. Knitted fabrics are rapidly produced by knitting and tend to be loose and elastic when being worn. Strands of fibers are interlocked by heat, moisture, pressure or striking to construct felt fabrics, thus eliminating the need for the use of threads. In plaited, braided and lace fabrics, individual threads are interlaced with sets of threads while sliding in any one direction to attain desired effects. Non-woven fabrics are constructed by the application of adhesive materials, the attachment of fibers through chemical functions on the surface of the fibers, or the attachment of webs or sheets of thermoplastic fibers by heating. Laminated fabrics are constructed by laminating a foam to one or two woven fabrics to achieve improved flexibility and provide a cushiony feeling. The surface areas of molded fabrics are larger than those of the raw materials before extrusion. Molded articles (e.g., clothes) are cushiony, or are in the form of a pile or plate. These articles are very wearable, match the functions of the human body, and are not readily deformed.

The lateral sides of two-dimensional fabrics are not utilized or used. Sewing and other fusion techniques are currently used to impart three-dimensional shapes to fabrics.

Industrial applications of such techniques have been reported. For example, U.S. Patent No. 3,384,519 suggests a blind comprising two-layered fabrics and a movable blade positioned between the fabrics wherein the fabrics and blade are adhered to the blade by fusion or bonding. The horizontal movement of the blade allows light to enter through the mesh type fabrics, and the vertical movement of the blade blocks light. By the movements of the blade, the amount of light entering the blind can be controlled. In addition, the soft texture and mesh structure of the fabrics enable the blind to shield light in a controllable manner. However, the use of an adhesive or pressure-sensitive adhesive for the adhesion of the blade to the fabrics may cause the problems of indoor environmental pollution. Particularly, long-term use of the blind causes a deterioration in the physical properties of the adhesive or pressure-sensitive adhesive by UV light, resulting in poor adhesion between the blade and the fabrics. In serious cases, the blade is separated from the fabrics.

In an attempt to overcome the above problems, a three-dimensional fabric is suggested in WO 2008/127030 A1. The three-dimensional fabric includes a surface layer, a backing layer, and an intermediate layer connecting the surface layer and the backing layer. The intermediate layer is composed of first intermediate portions and second intermediate portions. The surface layer includes sequential unstitched surface portions and sequential stitched surface portions formed in an alternating and repeating pattern. The unstitched surface portions are essentially composed of surface warp threads only and the stitched surface portions are composed of the surface warp threads and intermediate warp threads. The backing layer includes sequential unstitched backing portions and sequential stitched backing portions formed in an alternating and repeating pattern. The unstitched backing portions are essentially composed of backing warp threads only and the stitched backing portions are composed of the backing warp threads and the intermediate warp threads. The intermediate layer includes sequential intermediate portions composed of the intermediate warp threads only and connected to the stitched surface portions composed of the intermediate warp threads only and connected to the stitched surface portions and the stitched backing portions in an alternating and repeating pattern.

The greatest problem of the patent is that the intermediate portions of the three-dimensional fabric have a single-layer structure, so that it is impossible for light to be shield completely. Therefore, the patented fabric is not applicable in various fields such as movie theaters, lecture rooms, presentation rooms, laboratories, and so forth in which light should be shield perfectly.

Further, GB 722 090 A discloses a webbing for venetian blinds, with cross threads in between main bandings, wherein some only of the warp threads of the strap may be woven, the remainder of the warp threads being weftless. Furthermore, EP 0 447 058 A1, EP 0 733 730 A2 and FR 2 907 475 A1 disclose three-dimensional fabrics comprising several fabric layers.

The present invention has been made in an effort to solve the above problems, and it is an object of the present invention to provide fabrics that can be woven on a single loom in a batch operation by novel weaving techniques and undergo transformation between two-dimensional and three-dimensional shapes, and are applicable as materials for blinds with high light-shielding rate due to intermediate portions having a multi-layered structure and, and methods for the production of the fabrics.

The present invention provides a three-dimensional multilayer fabric according to claim 1.

Embodiments of the present invention provide a three-dimensional multilayer fabric comprising a surface layer, a backing layer and an intermediate layer connecting the surface layer and the backing layer wherein the intermediate layer has a multi-layered structure where multiple fabric layers are separated from each other and is composed of first intermediate portions and second intermediate portions, the surface layer includes sequential unstitched surface portions and sequential stitched surface portions formed in an alternating and repeating pattern, the unstitched surface portions being composed of surface warp threads only and the stitched surface portions being composed of the surface warp threads and intermediate warp threads; the backing layer includes sequential unstitched backing portions and sequential stitched backing portions formed in an alternating and repeating pattern, the unstitched backing portions being composed of backing warp threads only and the stitched backing portions being composed of the backing warp threads and the intermediate warp threads; and the intermediate layer includes sequential intermediate portions composed of the intermediate warp threads only and connected to the stitched surface portions and the stitched backing portions in an alternating and repeating pattern, the intermediate warp threads being woven without interlacing with weft threads on the surfaces of the unstitched backing portions and exposed to the outside, followed by shearing.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other and is composed of first intermediate portions and second intermediate portions, the surface layer includes sequential unstitched surface portions and sequential stitched surface portions formed in an alternating and repeating pattern, the unstitched surface portions being composed of surface warp threads only and the stitched surface portions being composed of the surface warp threads and intermediate warp threads; the backing layer includes sequential unstitched backing portions and sequential stitched backing portions formed in an alternating and repeating pattern, the unstitched backing portions being composed of backing warp threads only and the stitched backing portions being composed of the backing warp threads and the intermediate warp threads; and the intermediate layer includes sequential intermediate portions composed of the intermediate warp threads only and connected to the stitched surface portions and the stitched backing portions in an alternating and repeating pattern, the intermediate warp threads being woven without interlacing with weft threads on the surfaces of the unstitched backing portions and the unstitched surface portions and exposed to the outside, followed by shearing.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other and is composed of first intermediate portions and second intermediate portions, the surface layer includes sequential unstitched surface portions and sequential stitched surface portions formed in an alternating and repeating pattern, the unstitched surface portions being composed of surface warp threads only and the stitched surface portions being composed of the surface warp threads and intermediate warp threads; the backing layer includes sequential unstitched backing portions and sequential stitched backing portions formed in an alternating and repeating pattern, the unstitched backing portions being composed of backing warp threads and the intermediate warp threads; and the intermediate layer includes sequential intermediate portions composed of the intermediate warp threads only and connected to the stitched surface portions and the stitched backing portions in an alternating and repeating pattern, the intermediate warp threads being interlaced with extra weft threads on the surface layer to form protruding portions exposed on a surface of a fabric, after which the protruding portions are removed to create a three-dimensional shape.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other, the surface layer includes sequential unstitched surface portions and sequential stitched surface portions formed in an alternating and repeating pattern, the unstitched surface portions being composed of surface warp threads only and the stitched surface portions being composed of the surface warp threads and a part of intermediate warp threads; the backing layer includes sequential unstitched backing portions and sequential stitched backing portions formed in an alternating and repeating pattern, the unstitched backing portions being composed of backing warp threads only and the stitched backing portions being composed of the backing warp threads and extra warp threads being not composed of the stitched surface portions; and the intermediate layer includes sequential intermediate portions composed of the intermediate warp threads only and connected to the stitched surface portions and the stitched backing portions in an alternating and repeating pattern, connecting warp threads of the intermediate layer connecting the stitched surface portions and the stitched backing portions being sheared.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other and is composed of first intermediate portions and second intermediate portions and the surface layer and the backing layer are composed of their respective stitched portions where unstitched surface portions and unstitched backing portions are in contact with the intermediate layer, the surface layer and the backing layer are formed of two more warp threads and the first and second intermediate portions are composed of four more even- numbered warp threads, the unstitched surface portions and the unstitched backing portions are formed of two more warp threads, first and third stitched surface portions are formed of warp threads of the unstitched surface portions and warp threads of the first intermediate portions and second stitched surface portions are formed of warp threads of the unstitched surface portions and warp threads of the second intermediate portions, first and third stitched backing portions are formed of warp threads of the unstitched backing portions and warp threads of the second intermediate portions and the second stitched backing portions are formed of warp threads of the unstitched backing portions and warp threads of the first intermediate portions, the first and second intermediate portions are formed of two more warp threads to separate a multiple of a fabric, connecting warp threads of the intermediate layer exposed to the outside of the backing layer are sheared.

In some embodiments of the present invention, when surface warp threads are 1/2, backing warp threads are 3/4, first intermediate warp threads are 5/6/7/8 and second intermediate warp threads are 9/10/11/12, as indicated by harness numbers, the unstitched surface portions and the unstitched backing portions are essentially composed of 1/2 and 3/4, respectively, the first and third stitched surface portions of the surface layer are composed of 1/2/5/6/7/8, and the second stitched surface portion is composed of 1/2/9/10/11/12, the first and third stitched backing portions of the baking layer are composed of 3/4/9/10/11/12, the second stitched backing portion is composed of 3/4/5/6/7/8, and the first intermediate portions form one fabric layer using 5/6 and the other fabric layer using 7/8 to separate them each other, and the second intermediate portions form one fabric layer using 9/10 and the other fabric layer using 11/12 to separate them each other.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other and is composed of first intermediate portions and second intermediate portions and the surface layer and the backing layer are composed of their respective stitched portions where unstitched surface portions and unstitched backing portions are in contact with the intermediate layer, the surface layer and the backing layer are formed of two more warp threads and the first and second intermediate portions are composed of four more even- numbered warp threads, the unstitched surface portions are formed of two more warp threads, the first and second intermediate portions are formed of two more warp threads to separate a multiple of a fabric, first and third stitched backing portions are formed of warp threads of the unstitched backing portions and warp threads of the second intermediate portions and the second stitched backing portions are formed of warp threads of the unstitched backing portions and warp threads of the first intermediate portions, the unstitched backing portion till the first stitched backing portion and the stitched portion are composed of warp threads of the backing layer and warp threads of the second intermediate portions, the unstitched backing portion till the second stitched backing portion and the stitched portion are composed of warp threads of the backing layer and warp threads of the first intermediate portions, the unstitched backing portion till the third stitched backing portion and the stitched portion are composed of warp threads of the backing layer and warp threads of the second intermediate portions, the above procedure is sequentially repeated, and protruding portions exposed to the outside of the surface layer are removed.

In some embodiments of the present invention, when surface warp threads are 1/2, backing warp threads are 3/4, first intermediate warp threads are 5/6/7/8 and second intermediate warp threads are 9/10/11 /12, as indicated by harness numbers, the unstitched surface portions are essentially composed of 1/2, the first intermediate portions form one fabric layer using 5/6 and the other fabric layer using 7/8 to separate them each other, and the second intermediate portions form one fabric layer using 9/10 and the other fabric layer using 11/12 to separate them each other, the first and third stitched surface portions of the surface layer are composed of 1/2/5/6/7/8, and the second stitched surface portion is composed of 1/2/9/10/11/12, the first and third stitched backing portions of the baking layer are composed of 3/4/9/10/11/12, the second stitched backing portion is composed of 3/4/5/6/7/8, the unstitched backing portion till the first stitched backing portion and the stitched portion are composed of 3/4/9/10/11/12, the unstitched backing portion till the second stitched backing portion and the stitched portion are composed of 3/4/5/6/7/8, the unstitched backing portion till the third stitched backing portion and the stitched portion are composed of 3/4/9/10/11/12, the above procedure is sequentially repeated.

Embodiments of the present invention provide a three-dimensional multilayer fabric, comprising a surface layer, a backing layer and an intermediate layer connecting the surface layer and the backing layer wherein the intermediate layer has a multi-layered structure where multiple fabric layers are separated from each other and the surface layer and the backing layer are composed of their respective stitched portions where unstitched surface portions and unstitched backing portions are in contact with the intermediate layer, the surface layer and the backing layer are formed of two more warp threads and intermediate portions are composed of four more even- numbered warp threads, the unstitched surface portions and the unstitched backing portions are formed of two more warp threads, the intermediate portions are formed of two more warp threads to separate a multiple of a fabric, the stitched surface portions are composed of surface warp threads and a part of warp threads of fabric layers, the stitched backing portions are composed of backing warp threads and extra fabric layers, except for the warp threads of the fabric layers being composed of the stitched surface portions, connecting warp threads connecting the stitched surface portions and stitched backing portions are sheared.

In some embodiments of the present invention, when surface warp threads are 1/2, backing warp threads are 3/4, intermediate warp threads are 5/6/7/8, as indicated by harness numbers, the unstitched surface portions are essentially composed of 1/2 and the unstitched backing portions are essentially composed of 3/4, the intermediate portions form one fabric layer using 5/6 and the other fabric layer using 7/8 to separate them each other, the stitched surface portions are essentially composed of 1/2/6/8, the stitched backing portions are essentially composed of 3/4/5/7.

In other embodiments of the present invention, the warp thread and/or the weft thread is woven with a low-melting point yarn.

In further embodiments of the present invention, the low-melting point yarn is a grey yarn whose melting point is intentionally lowered by one more method selected from the group consisting of modification of molecular structure, copolymerization, blending, spinning process control or composite spinning so that the surface is allowed to be minutely fused by thermal treatment in the temperature range of about 120°C to about 190°C.

In other embodiments of the present invention, the warp thread and/or the weft thread is a grey yarn in which a low-melting point yarn and a flame-retardant yarn are mixed or a composite fiber composed of low-melting point portions and flame-retardant portions.

In yet other embodiments of the present invention, the fabric is further thermally treated to achieve improved shape stability and enhanced stiffness.

In further embodiments of the present invention, the surface layer and the backing layer are formed into a mesh structure by weaving.

In other embodiments of the present invention, the intermediate layer is denser than the surface layer and the backing layer.

In further embodiments of the present invention, a cloth is provided using the three-dimensional multilayer fabric.

In yet further embodiments of the present invention, an article is provided using the three-dimensional multilayer fabric.

In other embodiments of the present invention, a blind is provided using the three-dimensional multilayer fabric.

### [Advantageous Effects]

The fabrics and the methods according to the embodiments of the present invention have the following advantageous effects.

The fabrics can be transformed from two-dimensional shape to and three-dimensional shape according to a conventional weaving method. The three-dimensional multilayer fabric according to the present invention can shield light perfectly due to intermediate portions having a multi-layered structure so that it is applicable in various fields such as movie theaters, lecture rooms, presentation rooms, laboratories, and so forth in which light should be shield perfectly.

Additionally, the design, color depth and light-shielding effects of the fabrics can be effectively varied through the transformation between two-dimensional and three-dimensional shapes.

### [Description of Drawings]

FIG. 1 is a cross-sectional view of a fabric according to a preferred embodiment of the present invention along the running direction of warp threads;
FIG. 2 is a conceptual sectional view illustrating the production of the fabric according to a first embodiment of the present invention;
FIG. 3 is a conceptual sectional view illustrating the production of the fabric as indicated by harness numbers according to a first embodiment of the present invention;
FIG. 4 is a conceptual sectional view illustrating the production of the fabric according to a second embodiment of the present invention;
FIG. 5 is a cross-sectional view of the fabric according to a third embodiment of the present invention along the running direction of warp threads;
FIG. 6 is a conceptual sectional view illustrating the production of the fabric as indicated by harness numbers according to the third embodiment of the present invention;
FIG. 7 is a cross-sectional view of the fabric according to a fourth embodiment of the present invention along the running direction of warp threads;
FIG. 8 is a conceptual sectional view illustrating the production of the fabric as indicated by harness numbers according to the fourth embodiment of the present invention; and
FIG. 9 is a flow chart illustrating the production of the fabric according to the embodiments of the present invention.

**<Brief explanation of essential parts of the drawings>**

| | | | |
|---|---|---|---|
| 100: | Surface layer | 110: | Stitched surface portions |
| 120: | Unstitched surface portions | 200: | Backing layer |
| 210: | Stitched backing portions | 220: | Unstitched backing portions |
| 300: | Intermediate layer | 400: | Protruding portions |

### [Best Mode]

Preferred embodiments of the present invention will now be described in detail with reference to the accompanying drawings. It should be noted that whenever possible, the same reference numerals will be used throughout the drawings and the description to refer to the same or like parts. In describing the present invention, detailed descriptions of related known functions or configurations are omitted in order to avoid making the essential subject of the invention unclear.

As used herein, the terms "about", "substantially", etc. are intended to allow some leeway in mathematical exactness to account for tolerances that are acceptable in the trade and to prevent any unconscientious violator from unduly taking advantage of the disclosure in which exact or absolute numerical values are given so as to help understand the invention.

The term "fabrics" is defined to include woven fabrics, knitted fabrics, felt fabrics, plaited fabrics, non-woven fabrics, laminated fabrics and molded fabrics. Woven fabrics are exemplified in order to better understand the embodiments of the present invention. Thus, it is to be understood that the woven fabrics are produced by the interlacing of warp threads and weft threads. The expression "warp threads only are woven" is used herein to mean that the warp threads are interlaced with weft threads, but the expression 'not interlaced with weft threads' is not applied thereto.

The three-dimensional multilayer fabric can be formed in a three-layered structure. In actuality, the fabrics are formed as illustrated FIG. 1, for convenience of explanation, a surface layer 100 and a backing layer 200 are separated as shown FIGs. 2 to 8.

FIG. 1 is a cross-sectional view of a fabric according to a preferred embodiment of the present invention along the running direction of warp threads. FIG. 2 is a conceptual sectional view illustrating the production of the fabric according to a first embodiment of the present invention. FIG. 3 is a conceptual sectional view illustrating the production of the fabric as indicated by harness numbers according to a first embodiment of the present invention. FIG. 4 is a conceptual sectional view illustrating the production of the fabric according to a second embodiment of the present invention. FIG. 5 is a cross-sectional view of the fabric according to a third embodiment of the present invention along the running direction of warp threads. FIG. 6 is a conceptual sectional view illustrating the production of the fabric as indicated by harness numbers according to the third embodiment of the present invention. FIG. 7 is a cross-sectional view of the fabric according to a fourth embodiment of the present invention along the running direction of warp threads. FIG. 8 is a conceptual sectional view illustrating the production of the fabric as indicated by harness numbers according to the fourth embodiment of the present invention. FIG. 9 is a flow chart illustrating the production of the fabric according to the embodiments of the present invention. The present invention will be described hereinafter along the running direction of warp threads.

The three-dimensional multilayer fabric according to the present invention comprises a surface layer 100, a backing layer 200 and an intermediate layer 300 connecting the surface layer 100 and the backing layer 200.

The surface layer 100 includes stitched surface portions 110 and unstitched surface portions 120 formed in an alternating and repeating pattern, and the backing layer 200 includes stitched backing portions 210 and unstitched backing portions 220 formed in an alternating and repeating pattern. The unstitched surface portions 120 and the unstitched backing portions 220 are composed of surface warp threads and backing warp threads only, respectively. The stitched surface portions 110 can be composed of the surface warp threads and intermediate warp threads. The stitched backing portions 210 can be composed of the backing warp threads and the intermediate warp threads.

As shown in FIGs. 2 to 6, the intermediate layer includes a first intermediate portion and a second intermediate portion, which are only composed of different kinds of warp threads, repeatedly, i.e. first intermediate warp threads' and 'second intermediate warp threads', which are four more even-numbered warp threads. As show in FIGs. 7 and 8, the first intermediate portions are repeatedly formed to create the three-dimensional multilayer fabric.

The constituent intermediate warp threads of the intermediate layer are composed of four more even-numbered warp threads. For example, in case that two-layered fabric forms the intermediated layer, four warp threads are required at a minimum. As shown in FIG. 2, the first intermediate portions 310 and 312 composed of two-layered fabric and the second intermediate portions 320 and 322 are formed. Each of the fabric layer of the intermediate portions is separated from each other.

The three-dimensional multilayer fabric can be formed in various production methods. The fabrication procedure, as shown in FIG. 9. is carried out by the steps of forming the stitched surface portions, forming stitched backing portions, forming the unstitched surface layer, forming the intermediate layer, and forming the unstitched backing layer.

The unstitched surface portions 120 and the unstitched backing portions 220 are essentially composed of independent warp threads (*i.e.* the surface warp threads and the backing warp threads) in the first embodiment of the present invention of FIGs. 2 and 3. Starting from zone A of FIG. 2, the principle of weaving will be explained with regard to the formation of the layers using the respective warp threads. The surface warp threads are woven with the first intermediate warp threads forming the first intermediate portions 310 and 312 to form a first stitched surface portion 111. The first intermediate warp threads only are woven to form the first intermediate portion 310 and 312, and are then woven with the backing warp threads to form a second stitched backing portion 213 on the backing layer 200. Thereafter, the first intermediate warp threads are woven without interlacing with the weft threads and the backing warp threads only are woven to form the unstitched backing portion 220 in unstitched backing portions of zone B. The first intermediate warp threads (connecting warp threads 311) woven without interlacing the weft threads at the starting point of a third stitched surface portion 115 connect the starting point of a third stitched backing portion 215 to the starting point of the third stitched surface portion 115 and are woven together with the surface warp threads to form the third stitched surface portion 115. The subsequent procedure is carried out in the same manner as after the formation of the first stitched surface portion 111.

On the other hand, a first stitched backing portion 211 of the backing layer 200 is formed at the same vertical position as the first stitched surface portion 111. The backing layer 200 is essentially composed of the backing warp threads only. The first stitched backing portion 211 is composed of the backing warp threads and the second intermediate warp threads. Thereafter, the second intermediate warp threads are woven without interlacing the weft threads and the backing warp threads are interlaced with the weft threads to form the unstitched baking portion 220 (zone A). The second intermediate warp threads (connecting warp threads 321) woven without interlacing the weft threads are woven together with the surface warp threads at the starting point of the second stitched backing portion 213 to form a second stitched surface portion 113 of the surface layer 100. At this time, the connecting warp threads 321 serve to connect the second stitched surface portion 113 and the second stitched backing portions 213. Herein, the second stitched surface portion 113 may be formed at the same vertical position as the second stitched backing portion 213. The second intermediate warp threads having participated in the formation of the second stitched surface portion 113 are woven with only the second intermediate warp threads to form the intermediate layer (herein, the second intermediate portion in zone B) and are woven with the backing warp threads to form the third stitched backing portion 215. The subsequent procedure is carried out in the same manner as in zone A. The second intermediate portion is formed of the fabric layer separated the same as the first intermediate portion.

In FIG. 3, the method for weaving the fabric according to the present invention is simplified as indicated by harness numbers. As illustrated in FIG. 3, when the surface warp threads are 1/2, the backing warp threads are 3/4, the first intermediate warp threads are 5/6/7/8 and the second intermediate warp threads are 9/10/11/12, as indicated by harness numbers, the unstitched surface portions 120 and the unstitched backing portions 220 are essentially composed of 1/2 and 3/4, respectively, the first and third stitched surface portions of the surface layer 111 and 115 are composed of 1/2/5/6/7/8, and the second stitched surface portion 113 is composed of 1/2/9/10/11,12, the first and third stitched backing portions 211 and 215 of the backing layer are composed of 3/4/9/10/11/12, the second stitched backing portion 213 is composed of 3/4/5/6/7/8, and the first intermediate portions 310 and 312 are composed of 5/6/7/8. In addition, the first intermediate portions form one fabric layer using 5/6 and the other fabric layer using 7/8 to separate them each other. The second intermediate portions 320 and 322 are composed of 9/10/11/12 and the second intermediate portions form one fabric layer using 9/10 and the other fabric layer using 11/12 to separate them each other.

Referring to FIGs. 2 and 3, the production of the fabric according to the present invention will be explained in accordance with the actual weaving procedure. The first stitched surface portions 111 in zone A are started. That is, the surface warp threads and the first intermediate warp threads are once interlaced with the weft threads while shedding along a harness to form the first stitched surface portion 111. Thereafter, the backing warp threads and the second intermediate warp threads are interlaced with the weft threads during shedding to form the second stitched backing portion. This procedure is sequentially and repeatedly continued until the respective stitched portions are formed in accordance with the pre-designed length (for example, 1 cm) of the stitched portions.

After the formation of the stitched portions 111 and 211 is completed, the surface warp threads only are interlaced with the weft threads to form the unstitched surface portion 120 in zone A and the first intermediate warp threads only are interlaced with the weft threads to form the first intermediate portion. Further, only the backing warp threads are interlaced with the weft threads to form the unstitched backing portion 220. This procedure is sequentially and repeatedly continued as the pre-designed length just before the respective second stitched portions are formed.

The weaving in zone B is the same as in zone A except that different kinds of warp threads are used. The second intermediate warp threads are woven with the surface warp threads to form the second stitched surface portion 113 and the first intermediate warp threads are woven with the backing warp threads to form the second stitched backing portion 213. Thereafter, the surface warp threads are woven to form the unstitched surface portion, the second intermediate warp threads are woven to form the second intermediate portion 320, and the backing warp threads are woven to form the unstitched backing portion. These portions are formed sequentially and repeatedly by weaving in the same manner as in zone A.

The interlacing between the warp threads and the weft threads is basically conducted once, but the number of interlacing may vary in each layer depending on the fineness and texture of the warp/weft threads. In addition, the surface layer is first formed by weaving, but it should be understood that the intermediate layer or the backing layer can be formed before the surface layer.

The surface layer is connected to the backing layer by the connecting warp threads 311 and 321, thus making it impossible to create a three-dimensional shape. Accordingly, the removal of the connecting warp threads 311 and 321 is required to create a three-dimensional shape. FIG. 2 illustrates a state in which the connecting warp threads 311 and 321 are removed. By the removal of the connecting warp threads, the surface layer 100 and the backing layer 200 are connected to each other in an alternating manner through the intermediate layer 300. This alternating connection allows the fabric to create a three-dimensional shape. Specifically, the first stitched surface portion 111 is connected to the second stitched backing portion 213 through the first intermediate portion 310 and 312, and the second stitched surface portion 113 is connected to the third stitched backing portion 215 through the second intermediate portion 320 and 322. This structure may be repeated in a continuous pattern.

FIG. 4 is a conceptual sectional view illustrating the production of the fabric according to the second embodiment of the present invention. The basic principle of weaving is the same as in the fabric of the previous embodiment except that the connecting warp threads 311 and 321 are stitched at different points. First, the weaving in zone A will be explained. The second intermediate warp threads having participated in the formation of the first stitched backing portion 211 are woven without interlacing with the weft threads to form the unstitched backing portion 220 in sub-zone (a), as explained in the previous embodiment. In the first embodiment, the second intermediate warp threads are moved to the surface layer 100 and are woven together with the surface warp threads at the starting point of the second stitched backing portion 213 to form the second stitched surface portion 113. In the present embodiment, the second intermediate warp threads are moved from any point of the zone, where only the unstitched backing portion 220 is formed, to the surface layer 110, and then are woven without interlacing with the weft threads in sub-zone (b) of the unstitched surface portion 120 to form the second stitched surface portion 113. Thereafter, the second intermediate warp threads are woven together with surface warp threads in a zone where the second stitched surface portion 113 is formed, as described in the previous embodiment. The weaving of the first intermediate warp threads is also carried out in the same manner as in the previous embodiment.

Some of the warp threads that are not interlaced with the weft threads are exposed to the surfaces of the surface layer and the backing layer. In the first embodiment, some of the warp threads that are not interlaced with the weft threads are exposed to only the surface of the backing layer.

Since the surface layer is connected to the backing layer by the connecting warp threads 311 and 321 according to the first and second embodiments, the removal of the connecting warp threads 311 and 321 is required to create a three-dimensional shape. The fabric of the present embodiment has the advantage that the introduction of the connecting warp threads arising from the random movement of fibers after cutting can be prevented.

The connecting warp threads can be removed by various methods, for example, shearing. Specifically, some of the warp threads exposed from the backing layer 200 without interlacing with the weft threads can be cut and removed by suction.

FIGs. 5 to 6 illustrate a fabric according to the third embodiment of the present invention. The weaving and the basic structure of the fabric are the same as the foregoing embodiments except that the intermediate warp threads run in different directions during weaving.

First, the surface warp threads are woven without interlacing with the other warp threads to form the unstitched surface portion 120 of the surface layer 100 and are then woven with the second intermediate warp threads to form the second stitched surface portion 113 in zone A. The formation of the second intermediate portion 320 by weaving only the second intermediate warp threads is the same as in the foregoing embodiments. Thereafter, the connecting warp threads 321 of the second intermediate portion 320 are exposed to the surface of the surface layer to form protruding portions 400. As illustrated in the enlarged partial view of the FIG. 5, two weft threads are woven upwardly and downwardly with respect to the warp threads 321 to surround the warp threads 321. The connecting warp threads 321 interlaced with the weft threads are woven together with the backing warp threads to form the backing layer 200 and are woven together with the backing warp threads to form the third stitched backing portion 215 in zone B. Again, the backing warp threads are woven together with the first intermediate warp threads to form the backing layer 200 and are then woven with the first intermediate warp threads to form the second stitched backing portion 213 in zone A. Thereafter, the first intermediate warp threads are woven to form the first intermediate portion 310, woven with the surface warp threads to form the third stitched surface portion 115 and woven with extra weft threads to form protruding portions 400 exposed to the surface of the third stitched surface portion 115 in zone B. The first intermediate warp threads are woven with the backing warp threads to form the backing layer after the third stitched backing portion 215. That is, in the present embodiment, the first or second intermediate warp threads are woven with the backing warp threads to form the unstitched backing portions 220 and the stitched backing portions 210 of the backing layer, and the second or first intermediate warp threads are woven with the backing warp threads to form the unstitched backing portions 220 and the stitched backing portions 210 of the backing layer in an alternating and repeating pattern in the other zone.

In FIG. 6, the method for weaving the fabric according to the present invention is simplified as indicated by harness numbers. As illustrated in FIG. 6, when the warp threads of the surface layer 100 are 1/2, the warp threads of the backing layer 200 are 3/4, the warp treads of the first intermediate portion 310 are 5/6/7/8 and the warp treads of the second intermediate portion 320 are 9/10/11/12, as indicated by harness numbers, the surface layer 100 are essentially composed of 1/2, the first and third stitched surface portions of the surface layer 111 and 115 are composed of 1/2/5/6/7/8, and the second stitched surface portion 113 is composed of 1/2/9/10/11,12. The unstitched backing portion till the first stitched backing portion 211 and the stitched portion are composed of 3/4/9/10/11/12. The unstitched backing portion till the second stitched backing portion 213 and the stitched portion are composed of 3/4/5/6/7/8, the unstitched backing portion till the third stitched backing portion 215 and the stitched portion are composed of 3/4/9/10/11/12. The above procedure is sequentially repeated. The first and second intermediate portions are composed of 5/6/7/8 and 9/10/11/12, respectively.

Since the surface layer is connected to the backing layer by the connecting warp threads 311 and 321, it is necessary to remove the connecting warp threads. As mentioned earlier, the connecting warp threads can be removed by shearing. Alternatively, the connecting warp threads can be removed in a more convenient manner by removing the warp threads 400 exposed to the surface layer. That is, the connecting warp threads exposed to the surface layer are fixed by the weft threads. The weft threads are continuously exposed together with the connecting warp threads in the width direction. When it is intended to move upwardly and remove the weft threads exposed to the surface laver, the connecting warp threads interlaced together with the weft threads are also moved upwardly and cut at the respective stitched portions. As a result, the connecting warp threads can be completely removed together with the weft threads.

FIGs. 7 to 8 illustrate a fabric according to the fourth embodiment of the present invention. In previous first to third embodiments, the intermediate portions are composed of the first and second intermediate portions. That is, the three-dimensional multilayer fabric is formed employing the intermediate portions having different warp threads and being repeated. In this method, there are several warp threads not woven with the weft threads and sheared warp threads, so that procedure can be complex.

In the fourth embodiment, the weaving and the basic structure of the fabric such that the surface layer, the backing layer, and the intermediate layer having a multi-layered structure where a multiple of fabrics are separated each other, are the same as the foregoing embodiments except that the warp threads composed of the stitched portions.

The unstitched surface portions 120 and the unstitched backing portions 220 are essentially composed of independent warp threads.

The stitched surface portions 110 are composed of the warp threads of the unstitched surface portions 120 and a part of the warp threads of the intermediate portions 310 and 312. The stitched backing portions 210 are composed of the warp threads of the unstitched backing portions 220 and extra warp threads being not composed of the stitched surface portions 110 among the warp threads composed of the intermediate portions 310 and 312. In the event that the fabric layer is composed of two warp threads, one is composed of the stitched surface portions and the other is composed of the stitched backing portions.

The warp threads composed of the stitched surface portions 110 form the intermediate portions and form prior connecting warp threads 313 connecting the stitched surface portions 110 without the weft threads at a starting point of the stitched backing portion 210 and then form the stitched surface portions 110 together with the warp threads of the unstitched surface portions 120.

The warp threads composed of the stitched backing portions 210 are woven with the warp threads of the unstitched backing portion 220 to form the stitched backing portions 210 and form a post connecting warp threads 315 connecting the stitched surface portions 110 without the weft threads at an end point of the stitched backing portion 210 and then form the intermediate portions 310 and 312.

In FIG. 8, the method for weaving the fabric according to the present invention is simplified as indicated by harness numbers. As illustrated in FIG. 8, when the surface warp threads are 1/2, the backing warp threads are 3/4, the first intermediate warp threads are 5/6/7/8, as indicated by harness numbers, the unstitched surface portions 120 and the unstitched backing portions 220 are essentially composed of 1/2 and 3/4, respectively, the stitched surface portions 110 are composed of 1/2/6/8, and the stitched backing portions 210 are composed of 3/4/5/7. In addition, the intermediate portions 310 and 312 are composed of 5/6/7/8 and the intermediate portions form one fabric layer using 5/6 and the other fabric layer using 7/8 to separate them each other.

The procedure according to the fourth embodiment is simple as compared to the first to third embodiments as aforementioned. The three-dimensional multiplayer fabric according to the fourth embodiment has advantages that there is no warp threads exposed to the outside of the surface layer and the backing layer and the protrusion portions are not formed while two connecting warp threads for connecting the stitched surface portions and the stitched backing portions are formed.

In the fabrics according the fourth embodiment, since the stitched surface portions are combined with the stitched backing portions by the prior and post connecting warp threads 313 and 315, it is necessary to remove the prior and post connecting warp threads 313 and 315 in order to embody three-dimensional shape

The fabric may be thermally treated before or after the shearing to achieve improved shape stability and enhanced stiffness. The thermal treatment is preferably carried out before shearing to make the fabric stiffer. When the thermal treatment is carried out after shearing, an excessive stress (*e.g.*, cutting) is applied to the fabric in the state where the multiple layers are adhered, and as a result, the fabric may be damaged.

To avoid damage to the fabric, the warp thread and/or the weft thread is woven with a low-melting point yarn. As the low-melting point yarn, there may be used a grey yarn whose melting point is intentionally lowered by modification of molecular structure, copolymerization, blending, spinning process control or composite spinning so that the surface can be minutely fused by thermal treatment in the temperature range of about 120°C to about 190°C. Specifically, as the grey yarn, Korean Patent No. 289414 suggests a copolyester-based binder fiber prepared by copolymerizing terephthalic acid or its ester-forming derivative, ethylene glycol and neopentyl glycol. Further, the low-melting yarn produced by composite spinning is composed of a core portion and a sheath portion. The core portion serves as a support and the sheath portion is fused during thermal treatment. As the low-melting yarn, Korean Patent No. 587122 suggests a heat-fusible composite fiber comprising a low-melting point ingredient and a high-melting point ingredient wherein the low-melting point ingredient forms continuously at least a part of the fiber surface in the fiber direction, has a glass transition temperature higher than 60°C and is composed of a mixture of 1 to 20 wt% of polyolefin and 80 to 99 wt% of a copolyester having 50 to 70 mol% of polyethylene terephthalate units.

As the warp thread and/or the weft thread, there can be used a mixture in which a low-melting point yarn and a flame-retardant yarn are mixed, a composite fiber (*e.g.,* sheath-core type, split type, multiple sea-island type, etc.) composed of a low-melting point portion and a flame-retardant portion, or a blended spun yarn of a low-melting point yarn and a flame retardant yarn. In this case, the fabrics can be utilized as industrial materials, particularly, curtain sheets and blinds. At this time, the ratio between the low-melting point portion and the flame-retardant portion or between the low-melting point yarn and the flame-retardant yarn is preferably from 15:85 to 50:50 (w/w). When the flame retardant portion (or yarn) is present in the amount of less than 50 wt%, the flame retardance of the fabric is deteriorated. Meanwhile, when the flame retardant portion (or yarn) is present in the amount exceeding 85%, the degree of fusion of the flame retardant portion (or yarn) during thermal treatment is low, and as a result, improvement in the stiffness of the fabric is negligible.

In the fabrics according to the present invention, the surface laver, the backing layer and the intermediate layer may have different texture densities. For example, the surface laser and the backing layer are configured to have a mesh structure by weaving, and the intermediate layer is configured to be denser than the surface layer and the backing layer. When the fabric has a structure in which the inner and outer portions are not exposed, as illustrated in FIG. 1, it does not create a three-dimensional shape. When the fabric has a structure in which the intermediate layer is movable in the vertical direction with respect to the surface layer and the backing layer and the inner and outer portions of the layers are exposed due to the mesh structure of the surface layer and the backing layer, it can create a three-dimensional shape. This structure indicates that the fabric can be utilized as a material for light shielding or security. In addition, the fabric can impart new functions to clothes. When the warp threads and the weft threads in the surface layer and the backing layer are positioned at intervals of 0.2 to 2 mm, more desirable effects of the fabric can be attained. Further, it is to be appreciated that the texture structure and design of the surface layer, the backing layer and the intermediate layer can be varied.

## Claims

1. A three-dimensional multilayer fabric, comprising a surface layer (100), a backing layer (200) and an intermediate layer (300) connecting the surface layer (100) and the backing layer (200),
wherein the surface layer (100) includes sequential unstitched surface portions (120) and sequential stitched surface portions (110) formed in an alternating and repeating pattern, the unstitched surface portions (120) being composed of surface warp threads only, and the stitched surface portions (110) being composed of the surface warp threads and intermediate warp threads,
wherein the backing layer (200) includes sequential unstitched backing portions (220) and sequential stitched backing portions (210) formed in an alternating and repeating pattern, the unstitched backing portions (220) being composed of backing warp threads only or of backing warp threads and intermediate warp threads, and the stitched backing portions (210) being composed of the backing warp threads and intermediate warp threads, and wherein the intermediate layer (300) includes sequential intermediate portions (310, 312; 320, 322) each connected to one of the stitched surface portions (110) and one of the stitched backing portions (210), respectively, the sequential intermediate portions (310, 312, 320, 322) being composed of intermediate warp threads only,
**characterized in that**
the intermediate layer (300) has a multi-layered structure where multiple fabric layers are separated from each other, wherein each intermediate portion (310, 312; 320, 322) forms a first fabric layer and a second fabric layer which are separated from each other.

2. A three-dimensional multilayer fabric according to claim 1, wherein the multiple fabric layers are composed of first intermediate portions (310, 312) and second intermediate portions (320, 322); and the sequential intermediate portions (310, 312, 320, 322) are connected to the stitched surface portions (110) and the stitched backing portions (210) in an alternating and repeating pattern, wherein the intermediate warp threads, which connect the stitched surface portions (110) and the stitched backing portions (210) and which are woven without interlacing with weft threads and which do not compose the intermediate portions (310, 312, 320, 322), are sheared.

3. A three-dimensional multilayer fabric according to claim 1, wherein the multiple fabric layers are composed of first intermediate portions (310, 312) and second intermediate portions (320, 322); and the sequential intermediate portions are connected to the stitched surface portions (110) and the stitched backing portions (210) in an alternating and repeating pattern, wherein the intermediate warp threads, which connect the stitched surface portions (110) and the unstitched backing portions (220) and which do not compose the intermediate portions (310, 312; 320, 322), are removed.

4. A three-dimensional multilayer fabric according to claim 1, wherein the stitched surface portions (110) are composed of the surface warp threads and a part of intermediate warp threads; and the stitched backing portions (210) are composed of the backing warp threads and another part of the intermediate warp threads which do not compose the stitched surface portions (110); and the sequential intermediate portions (310, 312, 320, 322) are connected to the stitched surface portions (110) and the stitched backing portions (210) in an alternating and repeating pattern, wherein connecting warp threads (313,315) of the intermediate layer (300) which connected the stitched surface portions (110) and the stitched backing portions (210), respectively, are sheared.

5. A three-dimensional multilayer fabric according to claim 1, wherein the multiple fabric layers are composed of first intermediate portions (310, 312) and second intermediate portions (320, 322) and the surface layer (100) and the backing layer (200) are composed of their respective stitched portions (110, 210) where unstitched surface portions (120) and unstitched backing portions (220) are in contact with the intermediate layer (300), the surface layer (100) and the backing layer (200) are formed of at least two warp threads and the first and second intermediate portions (310, 312, 320, 322) are composed of an even number of at least four warp threads, the unstitched surface portions (120) and the unstitched backing portions (220) are formed of at least two warp threads, first and third stitched surface portions (111, 115) are formed of warp threads of the unstitched surface portions (120) and warp threads of the first intermediate portions (310, 312) and second stitched surface portions (113) are formed of warp threads of the unstitched surface portions (120) and warp threads of the second intermediate portions (320, 322), first and third stitched backing portions (211, 215) are formed of the warp threads of unstitched backing portions (220) and warp threads of the second intermediate portions (320, 322) and the second stitched backing portions (213) are formed of warp threads of the unstitched backing portions (220) and warp threads of the first intermediate portions (310, 312), the first and second intermediate portions (310, 312, 320, 322) are formed of at least two warp threads to separate multiple fabric layers, wherein connecting warp threads of the intermediate layer (300) are sheared.

6. The three-dimensional multilayer fabric according to claim 5, wherein when surface warp threads are first and second warp threads (1, 2), backing warp threads are third and fourth warp threads (3, 4), first intermediate warp threads are fifth, sixth, seventh, and eighth warp threads (5, 6, 7, 8) and second intermediate warp threads are ninth, tenth, eleventh and twelfth warp threads (9, 10, 11, 12), as indicated by harness numbers, the unstitched surface portions (120) and the unstitched backing portions (220) are essentially composed of the first and second warp threads (1, 2) and the third and fourth warp threads (3, 4), respectively, the first and third stitched surface portions (111, 115) of the surface layer (100) are composed of the first, second, fifth, sixth, seventh, and eighth warp threads (1, 2, 5, 6, 7, 8), and the second stitched surface portion (113) is composed of the first, second, ninth, tenth, eleventh, and twelfth warp threads (1, 2, 9, 10, 11, 12), the first and third stitched backing portions (211, 215) of the backing layer (200) are composed of the third, fourth, ninth, tenth, eleventh, and twelfth warp threads (3, 4, 9, 10, 11, 12), the second stitched backing portion (213) is composed of the third, fourth, fifth, sixth, seventh, and eighth warp threads (3, 4, 5, 6, 7, 8), and the first intermediate portions (310, 312) form one fabric layer using the fifth and sixth warp threads (5, 6) and the other fabric layer using the seventh and eighth warp threads (7, 8) to separate them each other, and the second intermediate portions 320, 322 form one fabric layer using the ninth and tenth warp threads (9, 10) and the other fabric layer using the eleventh and twelfth warp threads (11, 12) to separate them from each other.

7. A three-dimensional multilayer fabric according to claim 1, wherein the multiple fabric layers are composed of first intermediate portions (310, 312) and second intermediate portions (320, 322) and the surface layer (100) and the backing layer (200) are composed of their respective stitched portions (110, 210) where unstitched surface portions (120) and unstitched backing portions (220) are in contact with the intermediate layer (300), the surface layer (100) and the backing layer (200) are formed of at least two warp threads and the first and second intermediate portions (310, 312, 320, 322) are composed of an even number of at least four warp threads, the unstitched surface portions (120) are formed of at least two warp threads, the first and second intermediate portions (310, 312, 320, 322) are formed of at least two warp threads to separate multiple fabric layers, first and third stitched backing portions (211, 215) are formed of warp threads of the unstitched backing portions (220) and warp threads of the second intermediate portions (320, 322) and the second stitched backing portions (213) are formed of warp threads of the unstitched backing portions and warp threads of the first intermediate portions (310, 312), the unstitched backing portion (220) till the first stitched backing portion (211) and the stitched portion are composed of warp threads of the backing layer (200) and warp threads of the second intermediate portions (320, 322), the unstitched backing portion (220) till the second stitched backing portion (213) and the stitched portion are composed of warp threads of the backing layer (200) and warp threads of the first intermediate portions (310, 312), the unstitched backing portion (220) till the third stitched backing portion (215) and the stitched portion are composed of warp threads of the backing layer (200) and warp threads of the second intermediate portions (320, 322), the above arrangement is sequentially repeated, wherein the warp threads of the first and second intermediate portions (310, 312; 320, 322) connecting the stitched surface portions (110) and the unstitched backing portions (220) and not composing the intermediate portions (310, 312; 320, 322), are removed.

8. The three-dimensional multilayer fabric according to claim 7, wherein when surface warp threads are first and second warp threads (1, 2), backing warp threads are third and fourth warp threads (3, 4), first intermediate warp threads are fifth, sixth, seventh and eighth warp threads (5, 6, 7, 8) and second intermediate warp threads are ninth, tenth, eleventh and twelfth warp threads (9, 10, 11, 12), as indicated by harness numbers, the unstitched surface portions (120) are essentially composed of the first and second warp threads (1, 2), the first intermediate portions (310, 312) form one fabric layer using the fifth and sixth warp threads (5, 6) and the other fabric layer using the seventh and eighth warp threads (7, 8) to separate them each other, and the second intermediate portions (320, 322) form one fabric layer using the ninth and tenth warp threads (9, 10) and the other fabric layer using the eleventh and twelfth warp threads (11, 12) to separate them each other, the first and third stitched surface portions (111, 115) of the surface layer (100) are composed of the first, second, fifth, sixth, seventh and eighth warp threads (1, 2, 5, 6, 7, 8), and the second stitched surface portion (113) is composed of the first, second, ninth, tenth, eleventh and twelfth warp threads (1, 2, 9, 10, 11, 12), the first and third stitched backing portions (211, 215) of the backing layer are composed of the third, fourth, ninth, tenth, eleventh and twelfth warp threads (3, 4, 9, 10, 11, 12), the second stitched backing portion (213) is composed of the third, fourth, fifth, sixth, seventh and eighth warp threads (3, 4, 5, 6, 7, 8), the unstitched backing portion (220) till the first stitched backing portion (211) and the stitched portion are composed of the third, fourth, ninth, tenth, eleventh and twelfth warp threads (3, 4, 9, 10, 11, 12), the unstitched backing portion (220) till the second stitched backing portion (213) and the stitched portion are composed of the third, fourth, fifth, sixth, seventh and eighth warp threads (3, 4, 5, 6, 7, 8), the unstitched backing portion (220) till the third stitched backing portion (215) and the stitched portion are composed of the third, fourth, ninth, tenth, eleventh and twelfth warp threads (3, 4, 9, 10, 11, 12), the above arrangement is sequentially repeated.

9. A three-dimensional multilayer fabric according to claim 1, wherein the surface layer (100) and the backing layer (200) are composed of their respective stitched portions (110, 210) where unstitched surface portions (120) and unstitched backing portions (220) are in contact with the intermediate layer (300), the surface layer (100) and the backing layer (200) are formed of at least two warp threads and the intermediate portions (310, 312, 320, 322) are composed of an even number of at least four warp threads, the unstitched surface portions (120) and the unstitched backing portions (220) are formed of at least two warp threads, the intermediate portions (310, 312, 320, 322) are formed of at least two warp threads to separate multiple fabric layers, the stitched surface portions (110) are composed of surface warp threads and a part of warp threads of the fabric layers, the stitched backing portions (210) are composed of backing warp threads and another part of the warp threads of the fabric layers, which do not compose the stitched surface portions (110), wherein connecting warp threads (313, 315) which connected the stitched surface portions (110) and stitched backing portions (210), respectively, are sheared.

10. The three-dimensional multilayer fabric according to claim 9, wherein when surface warp threads are first and second warp threads (1, 2), backing warp threads are third and fourth warp threads (3, 4), intermediate warp threads are fifth, sixth, seventh and eighth warp threads (5, 6, 7, 8), as indicated by harness numbers, the unstitched surface portions (120) are essentially composed of the first and second warp threads (1, 2) and the unstitched backing portions (220) are essentially composed of the third and fourth warp threads (3, 4), the intermediate portions (310, 312, 320, 322) form one fabric layer using the fifth and sixth warp threads (5, 6) and the other fabric layer using the seventh and eighth warp threads (7, 8) to separate them each other, the stitched surface portions (110) are essentially composed of the first, second, sixth and eighth warp threads (1, 2, 6, 8), the stitched backing portions (210) are essentially composed of the third, fourth, fifth and seventh warp threads (3, 4, 5, 7).

11. The three-dimensional multilayer fabric according to any one of claims 1 to 10, wherein the warp thread and/or the weft thread is woven with a low-melting point yarn in the form of a heat-fusible composite fiber comprising a low-melting point ingredient and a high-melting point ingredient wherein the low-melting point ingredient forms continuously at least a part of the fiber surface in the fiber direction, has a glass transition temperature higher than 60°C and is composed of a mixture of 1 to 20 wt% of polyolefin and 80 to 99 wt% of a copolyester having 50 to 70 mol% of polyethylene terephthalate units.

12. The three-dimensional multilayer fabric according to claim 11, wherein the low-melting point yarn is a grey yarn whose melting point is intentionally lowered so that the surface is allowed to be minutely fused by thermal treatment in the temperature range of about 120°C to about 190°C.

13. The three-dimensional multilayer fabric according to any one of claims 1 to 10, wherein the warp thread and/or the weft thread is a grey yarn in which a low-melting point yarn in the form of a heat-fusible composite fiber comprising a low-melting point ingredient and a high-melting point ingredient wherein the low-melting point ingredient forms continuously at least a part of the fiber surface in the fiber direction, has a glass transition temperature higher than 60°C and is composed of a mixture of 1 to 20 wt% of polyolefin and 80 to 99 wt% of a copolyester having 50 to 70 mol% of polyethylene terephthalate units, and a flame-retardant yarn are mixed or a composite fiber composed of low-melting point portions and flame-retardant portions.

14. The three-dimensional multilayer fabric according to claim 12, wherein the fabric is further thermally treated to achieve improved shape stability and enhanced stiffness.

15. The three-dimensional multilayer fabric according to any one of claims 1 to 10, wherein the surface layer (100) and the backing layer (200) are formed into a mesh structure by weaving.

16. The three-dimensional multilayer fabric according to any one of claims 1 to 10, wherein the intermediate layer (300) is denser than the surface layer (100) and the backing layer (200).

17. A cloth using the fabric according to any one of claims 1 to 10.

18. An article using the fabric according to any one of claims 1 to 10.

19. A blind using the fabric according to any one of claims 1 to 10.

## Patentansprüche

1. Dreidimensionaler mehrlagiger Stoff, umfassend eine Oberflächenlage (100), eine Trägerlage (200) und eine Zwischenlage (300), die die Oberflächenlage (100) und die Trägerlage (200) verbindet,
wobei die Oberflächenlage (100) sequentielle nicht vernähte Oberflächenabschnitte (120) und sequentielle vernähte Oberflächenabschnitte (110) umfasst, die in einem alternierenden und sich wiederholenden Muster ausgebildet sind, wobei die nicht vernähten Oberflächenabschnitte (120) lediglich aus Oberflächenkettfäden bestehen und die vernähten Oberflächenabschnitte (110) aus den Oberflächenkettfäden und Zwischenkettfäden bestehen,
wobei die Trägerlage (200) sequentielle nicht vernähte Trägerabschnitte (220) und sequentielle vernähte Trägerabschnitte (210) umfasst, die in einem alternierenden und sich wiederholenden Muster ausgebildet sind, wobei die nicht vernähten Trägerabschnitte (220) lediglich aus Trägerkettfäden oder aus Trägerkettfäden und Zwischenkettfäden bestehen und die vernähten Trägerabschnitte (210) aus den Trägerkettfäden und den Zwischenkettfäden bestehen und die Zwischenlage (300) sequentielle Zwischenabschnitte (310, 312; 320, 322) umfasst, die jeweils mit einem der vernähten Oberflächenabschnitte (110) bzw. einem der vernähten Trägerabschnitte (210) verbunden sind, wobei die sequentiellen Zwischenabschnitte (310, 312, 320, 322) lediglich aus Zwischenkettfäden bestehen,
**dadurch gekennzeichnet, dass** die Zwischenlage (300) einen mehrlagigen Aufbau hat, bei dem mehrere Stofflagen voneinander getrennt sind, wobei jeder Zwischenabschnitt (310, 312; 320, 322) eine erste Stofflage und eine zweite Stofflage bildet, die voneinander getrennt sind.

2. Dreidimensionaler mehrlagiger Stoff nach Anspruch 1, bei dem die zahlreichen Stofflagen aus den ersten Zwischenabschnitten (310, 312) und den zweiten Zwischenabschnitten (320, 322) bestehen; und die sequentiellen Zwischenabschnitte (310, 312, 320, 322) mit den vernähten Oberflächenabschnitten (110) und den vernähten Trägerabschnitten (210) in einem alternierenden und sich wiederholenden Muster verbunden sind, wobei die Zwischenkettfäden, die die vernähten Oberflächenabschnitte (110) und die vernähten Trägerabschnitte (210) verbinden und die ohne Verweben von Schussfäden verwebt sind und nicht die Zwischenabschnitte (310, 312, 320, 322) umfassen, gemeinsam genutzt werden.

3. Dreidimensionaler mehrlagiger Stoff nach Anspruch 1, bei dem die zahlreichen Stofflagen aus ersten Zwischenabschnitten (310, 312) und zweiten Zwischenabschnitten (320, 322) bestehen; und die sequentiellen Zwischenabschnitte mit den vernähten Oberflächenabschnitten (110) und den vernähten Trägerabschnitten (210) in einem alternierenden und wiederholenden Muster verbunden sind, wobei die Zwischenkettfäden, die die vernähten Oberflächenabschnitte (110) und die nicht vernähten Trägerabschnitte (220) verbinden und die nicht die Zwischenabschnitte (310, 312; 320, 322) bilden, entfernt sind.

4. Dreidimensionaler mehrlagiger Stoff nach Anspruch 1, bei dem die vernähten Oberflächenabschnitte (110) aus den Oberflächenkettfäden und einem Teil der Zwischenkettfäden bestehen; und die vernähten Trägerabschnitte (210) aus den Trägerkettfäden und einem weiteren Teil der Zwischenkettfäden bestehen, die nicht die vernähten Oberflächenabschnitte (110) bilden; und die sequentiellen Zwischenabschnitte (310, 312, 320, 322) mit den vernähten Oberflächenabschnitten (110) und den vernähten Trägerabschnitten (210) in einem alternierenden und sich wiederholenden Muster verbunden sind, wobei die verbindenden Kettfäden (313, 315) der Zwischenlage (300), die die vernähten Oberflächenabschnitte (110) bzw. die vernähten Trägerabschnitte (210) verbinden, gemeinsam genutzt werden.

5. Dreidimensionaler mehrlagiger Stoff nach Anspruch 1, bei dem die zahlreichen Stofflagen aus den ersten Zwischenabschnitten (310, 312) und den zweiten Zwischenabschnitten (320, 322) bestehen und die Oberflächenlage (100) sowie die Trägerlage (200) aus ihren jeweiligen vernähten Abschnitten (110, 210) bestehen, wobei nicht vernähte Oberflächenabschnitte (120) und nicht vernähte Trägerabschnitte (220) mit der Zwischenlage (300) in Kontakt sind, die Oberflächenlage (100) und die Trägerlage (200) aus wenigstens zwei Kettfäden bestehen und die ersten sowie die zweiten Zwischenabschnitte (310, 312, 320, 322) aus einer geradzahligen Anzahl von wenigstens vier Kettfäden bestehen, die nicht vernähten Oberflächenabschnitte (120) und die nicht vernähten Trägerabschnitte (220) aus wenigstens zwei Kettfäden bestehen, erste und dritte vernähte Oberflächenabschnitte (111, 115) aus Kettfäden der nicht vernähten Oberflächenabschnitte (120) und Kettfäden der ersten Zwischenabschnitte (310, 312) bestehen und zweite vernähte Oberflächenabschnitte (113) aus Kettfäden der nicht vernähten Oberflächenabschnitte (120) und Kettfäden der zweiten Zwischenabschnitte (320, 322) bestehen, erste und dritte vernähte Trägerabschnitte (211, 215) aus den Kettfäden nicht vernähter Trägerabschnitte (220) bestehen und die Kettfäden der zweiten Zwischenabschnitte (320, 322) sowie die zweiten vernähten Trägerabschnitte (213) aus Kettfäden der nicht vernähten Trägerabschnitte (220) und Kettfäden der ersten Zwischenabschnitte (310, 312) bestehen, wobei die ersten und zweiten Zwischenabschnitte (310, 312, 320, 322) aus wenigstens zwei Kettfäden bestehen, um zahlreiche Stofflagen zu trennen, und die verbindenden Kettfäden der Zwischenlage (300) gemeinsam genutzt werden.

6. Dreidimensionaler mehrlagiger Stoff nach Anspruch 5, bei dem, wenn die Oberflächenkettfäden erste und zweite Kettfäden (1, 2) sind, Trägerkettfäden dritte und vierte Kettfäden (3, 4) sind, erste Zwischenkettfäden fünfte, sechste, siebte und achte Kettfäden (5, 6, 7, 8) und zweite Zwischenkettfäden neunte, zehnte, elfte und zwölfte Kettfäden (9, 10, 11, 12) sind, wie es durch Harnischnummern gekennzeichnet ist, die nicht vernähten Oberflächenabschnitte (120) und die nicht vernähten Trägerabschnitte (220) im wesentlichen aus den ersten und den zweiten Kettfäden (1, 2) bzw. den dritten und vierten Kettfäden (3, 4) bestehen, die ersten und dritten vernähten Oberflächenabschnitte (111, 115) der Oberflächenlage (100) aus den ersten, zweiten, fünften, sechsten, siebten und achten Kettfäden (1, 2, 5, 6, 7, 8) bestehen und der zweite vernähte Oberflächenabschnitt (113) aus den ersten, zweiten, neunten, zehnten, elften und zwölften Kettfäden (1, 2, 9, 10, 11, 12) besteht, die ersten und dritten vernähten Trägerabschnitte (211, 215) der Trägerlage (200) aus den dritten, vierten, neunten, zehnten, elften und zwölften Kettfäden (3, 4, 9, 10, 11, 12) bestehen, der zweite vernähte Trägerabschnitt (213) aus den dritten, vierten, fünften, sechsten, siebten und achten Kettfäden (3, 4, 5, 6, 7, 8) besteht und die ersten Zwischenabschnitte (310, 312) eine Stofflage mit Hilfe der fünften und sechsten Kettfäden (5, 6) und die andere Stofflage mit Hilfe der siebten und achten Kettfäden (7, 8) bilden, um sie voneinander zu trennen, und die zweiten Zwischenabschnitte 320, 322 eine Stofflage mit Hilfe der neunten und zehnten Kettfäden (9, 10) und die andere Stofflage mit Hilfe der elften und zwölften Kettfäden (11, 12) bilden, um diese voneinander zu trennen.

7. Dreidimensionaler mehrlagiger Stoff nach Anspruch 1, bei dem die zahlreichen Stofflagen aus den ersten Zwischenabschnitten (310, 312) und den zweiten Zwischenabschnitten (320, 322) bestehen und die Oberflächenlage (100) sowie die Trägerlage (200) aus ihren jeweiligen vernähten Abschnitten (110, 210) bestehen, die nicht vernähten Oberflächenabschnitte (120) und die nicht vernähten Trägerabschnitte (220) mit der Zwischenlage (300) in Kontakt sind, die Oberflächenlage (100) und die Trägerlage (200) aus wenigstens zwei Kettfäden ausgebildet sind und die ersten sowie zweiten Zwischenabschnitte (310, 312, 320, 322) aus einer geraden Zahl von wenigstens vier Kettfäden bestehen, die nicht vernähten Oberflächenabschnitte (120) aus wenigstens zwei Kettfäden ausgebildet sind, die ersten und zweiten Zwischenabschnitte (310, 312, 320, 322) aus wenigstens zwei Kettfäden ausgebildet sind, um mehrere Stofflagen zu trennen, erste und dritte vernähte Trägerabschnitte (211, 215) aus Kettfäden der nicht vernähten Trägerabschnitte (220) und Kettfäden der zweiten Zwischenabschnitte (320, 322) ausgebildet sind und die zweiten vernähten Trägerabschnitte (213) aus Kettfäden der nicht vernähten Trägerabschnitte und Kettfäden der ersten Zwischenabschnitte (310, 312) ausgebildet sind, der nicht vernähte Trägerabschnitt (220) bis zu dem ersten vernähten Trägerabschnitt (211) und der vernähte Abschnitt aus Kettfäden der Trägerlage (200) und Kettfäden der zweiten Zwischenabschnitte (320, 322) bestehen, der nicht vernähte Trägerabschnitt (220) bis zu dem zweiten vernähten Trägerabschnitt (213) und der vernähte Abschnitt aus Kettfäden der Trägerlage (200) und Kettfäden der ersten Zwischenabschnitte (310, 312) bestehen, der nicht vernähte Trägerabschnitt (220) bis zu dem dritten vernähten Trägerabschnitt (215) und der vernähte Abschnitt aus Kettfäden der Trägerlage (200) und Kettfäden der zweiten Zwischenabschnitte (320, 322) bestehen und die obige Anordnung sequentiell wiederholt wird, wobei die Kettfäden der ersten und zweiten Zwischenabschnitte (310, 312; 320, 322), die die vernähten Oberflächenabschnitte (110) und die nicht vernähten Trägerabschnitte (220) verbinden und nicht die Zwischenabschnitte (310, 312; 320, 322) bilden, entfernt sind.

8. Dreidimensionaler mehrlagiger Stoff nach Anspruch 7, bei dem, wenn Oberflächenkettfäden erste und zweite Kettfäden (1, 2) sind, Trägerkettfäden dritte und vierte Kettfäden (3, 4) sind, erste Zwischenkettfäden fünfte, sechste, siebte und achte Kettfäden (5, 6, 7, 8) sind und zweite Zwischenkettfäden neunte, zehnte, elfte und zwölfte Kettfäden (9, 10, 11, 12) sind, wie es durch Harnischnummern gekennzeichnet ist, die nicht vernähten Oberflächenabschnitte (120) im wesentlichen aus den ersten und zweiten Kettfäden (1, 2) bestehen, die ersten Zwischenabschnitte (310, 312) eine Stofflage mit Hilfe der fünften und sechsten Kettfäden (5, 6) und die andere Stofflage mit Hilfe der siebten und achten Kettfäden (7, 8) ausbilden, um sie voneinander zu trennen, und die zweiten Zwischenabschnitte (320, 322) eine Stofflage mit Hilfe der neunten und zehnten Kettfäden (9, 10) und die andere Stofflage mit Hilfe der elften und zwölften Kettfäden (11, 12) ausbilden, um diese voneinander zu trennen, die ersten und dritten vernähten Oberflächenabschnitte (111, 115) der Oberflächenlage (100) aus den ersten, zweiten, fünften, sechsten, siebten und achten Kettfäden (1, 2, 5, 6, 7, 8) bestehen und der zweite vernähte Oberflächenabschnitt (113) aus den ersten, zweiten, neunten, zehnten elften und zwölften Kettfäden (1, 2, 9, 10, 11, 12) besteht, die ersten und dritten vernähten Trägerabschnitte (211, 215) der Trägerlage aus den dritten, vierten, neunten, zehnten, elften und zwölften Kettfäden (3, 4, 9, 10, 11, 12) bestehen, der zweite vernähte Trägerabschnitt (213) aus den dritten, vierten, fünften, sechsten, siebten und achten Kettfäden (3, 4, 5, 6, 7, 8) besteht, der nicht vernähte Trägerabschnitt (220) bis zu dem ersten vernähten Trägerabschnitt (211) und der vernähte Abschnitt aus den dritten, vierten, neunten, zehnten, elften und zwölften Kettfäden (3, 4, 9, 10, 11, 12) besteht, der nicht vernähte Trägerabschnitt (200) bis zu dem zweiten vernähten Trägerabschnitt (213) und der vernähte Abschnitt aus den dritten, vierten, fünften, sechsten, siebten und achten Kettfäden (3, 4, 5, 6, 7, 8) bestehen, der nicht vernähte Trägerabschnitt (220) bis zu dem dritten vernähten Trägerabschnitt (215) und der vernähte Abschnitt aus den dritten, vierten, neunten, zehnten, elften und zwölften Kettfäden (3, 4, 9, 10, 11, 12) bestehen und die obige Anordnung sequentiell wiederholt wird.

9. Dreidimensionaler mehrlagiger Stoff nach Anspruch 1, bei dem die Oberflächenlage (100) und die Trägerlage (200) aus ihren jeweiligen vernähten Abschnitten (110, 210) bestehen, wobei die nicht vernähten Oberflächenabschnitte (120) und die nicht vernähten Trägerabschnitte (220) mit der Zwischenlage (300) in Kontakt sind, die Oberflächenlage (100) und die Trägerlage (200) aus wenigstens zwei Kettfäden ausgebildet sind und die Zwischenabschnitte (310, 312; 320, 322) aus einer geradzahligen Anzahl von wenigstens vier Kettfäden bestehen, die nicht vernähten Oberflächenabschnitte (120) und die nicht vernähten Trägerabschnitte (220) aus wenigstens zwei Kettfäden ausgebildet sind, die Zwischenabschnitte (310, 312, 320, 322) aus wenigstens zwei Kettfäden ausgebildet sind, um mehrere Stofflagen zu trennen, die vernähten Oberflächenabschnitte (110) aus Oberflächenkettfäden und einem Teil von Kettfäden der Stofflagen bestehen, die vernähten Trägerabschnitte (210) aus Trägerkettfäden und einem weiteren Teil der Kettfäden der Stofflagen bestehen, die nicht die vernähten Oberflächenabschnitte (110) umfassen, wobei verbindende Kettfäden (313, 315), die die vernähten Oberflächenabschnitte (110) bzw. die vernähten Trägerabschnitte (210) verbinden, gemeinsam genutzt werden.

10. Dreidimensionaler mehrlagiger Stoff nach Anspruch 9, bei dem, wenn die Oberflächenkettfäden erste und zweite Kettfäden (1, 2) sind, Trägerkettfäden dritte und vierte Kettfäden (3, 4) sind und Zwischenkettfäden fünfte, sechste, siebte und achte Kettfäden (5, 6, 7, 8) sind, wie es mit Harnischnummern gekennzeichnet ist, die nicht vernähten Oberflächenabschnitte (120) im wesentlichen aus den ersten und zweiten Kettfäden (1, 2) bestehen und die nicht vernähten Trägerabschnitte (220) im wesentlichen aus den dritten und vierten Kettfäden (3, 4) bestehen, die Zwischenabschnitte (310, 312, 320, 322) eine Stofflage mit Hilfe der fünften und sechsten Kettfäden (5, 6) und die andere Stofflage mit Hilfe der siebten und achten Kettfäden (7, 8) ausbilden, um diese voneinander zu trennen, die vernähten Oberflächenabschnitte (110) im wesentlichen aus den ersten, zweiten, sechsten und achten Kettfäden (1, 2, 6, 8) bestehen und die vernähten Trägerabschnitte (210) im wesentlichen aus den dritten, vierten, fünften und siebten Kettfäden (3, 4, 5, 7) bestehen.

11. Dreidimensionaler mehrlagiger Stoff nach einem der Ansprüche 1 bis 10, bei dem der Kettfaden und/oder Schussfaden mit einem Garn niedrigen Schmelzpunktes in Gestalt einer wärmeschmelzbaren Verbundfaser gewebt ist, die einen Inhaltsstoff mit einem niedrigen Schmelzpunkt und einen Inhaltsstoff mit einem hohen Schmelzpunkt umfasst, wobei der Inhaltsstoff niedrigen Schmelzpunktes kontinuierlich wenigstens einen Teil der Faseroberfläche in der Faserrichtung bildet, eine Glasübergangstemperatur hat, die höher ist als 60°C, und aus einem Gemisch von 1 bis 20 Gew.-% Polyolefin und 80 bis 99 Gew.-% eines Copolyesters besteht, der 50 bis 70 Mol-% von Polyethylenterephtalat-Einheiten hat.

12. Dreidimensionaler mehrlagiger Stoff nach Anspruch 11, bei dem das Garn mit niedrigem Schmelzpunkt ein graues Garn ist, dessen Schmelzpunkt absichtlich derart abgesenkt ist, dass es der Oberfläche gestattet ist, durch Wärmebehandlung in dem Temperaturbereich von etwa 120°C bis 190°C fein geschmolzen zu werden.

13. Dreidimensionaler mehrlagiger Stoff nach einem der Ansprüche 1 bis 10, bei dem der Kettfaden und/oder der Schussfaden ein graues Garn, bei dem ein Garn niedrigen Schmelzpunktes in Gestalt einer wärmeschmelzbaren Verbundfaser, die einen Inhaltsstoff eines niedrigen Schmelzpunktes und einen Inhaltsstoff eines hohen Schmelzpunktes umfasst, wobei der Inhaltsstoff niedrigen Schmelzpunktes kontinuierlich wenigstens einen Teil der Faseroberfläche in der Faserrichtung ausbildet, eine Glasübergangstemperatur hat, die höher als 60°C ist und aus einem Gemisch von 1 bis 20 Gew.-% eines Polyolefins und 80 bis 99 Gew.-% eines Copolyesters besteht, der 50 bis 70 Mol-% von Polyethylenterephtalat-Einheiten hat, und ein flammhemmendes Garn gemischt sind, oder eine Verbundfaser ist, die aus Abschnitten eines niedrigen Schmelzpunktes und flammhemmenden Abschnitten besteht.

14. Dreidimensionaler mehrlagiger Stoff nach Anspruch 12, bei dem die Faser weiterhin wärmebehandelt ist, um eine verbesserte Formstabilität und einer höhere Steifigkeit zu erzielen.

15. Dreidimensionaler mehrlagiger Stoff nach einem der Ansprüche 1 bis 10, bei dem die Oberflächenlage (100) und die Trägerlage (200) zu einer Gewebestruktur durch Weben ausgebildet sind.

16. Dreidimensionaler mehrlagiger Stoff nach einem der Ansprüche 1 bis 10, bei dem die Zwischenlage (300) dichter ist als die Oberflächenlage (100) und die Trägerlage (200).

17. Tuch, bei dem der Stoff nach einem der Ansprüche 1 bis 10 verwendet wird.

18. Gegenstand, bei dem der Stoff nach einem der Ansprüche 1 bis 10 verwendet wird.

19. Abschirmung, bei der der Stoff nach einem der Ansprüche 1 bis 10 verwendet wird.

## Revendications

1. Tissu 3D multicouche, comportant une couche superficielle (100), une couche support (200) et une couche intermédiaire (300) reliant la couche superficielle (100) et la couche support (200),
où la couche superficielle (100) comporte des parties superficielles séquentielles non cousues (120) et des parties superficielles séquentielles cousues (110) alternant de manière répétitive, les parties superficielles non cousues (120) étant uniquement composées de fils de chaîne superficiels, et les parties superficielles cousues (110) étant composées de fils de chaîne superficiels et de fils de chaîne intermédiaires,
où la couche support (200) comporte des parties de support séquentielles non cousues (220) et des parties de support séquentielles cousues (210) alternant de manière répétitive, les parties de support non cousues (220) étant uniquement composées de fils de chaîne de support ou bien de fils de chaîne de support et de fils de chaîne intermédiaires, et les parties de support cousues (210) étant composées des fils de chaîne de support et des fils de chaîne intermédiaires, et
où la couche intermédiaire (300) comporte des parties intermédiaires séquentielles (310, 312, 320, 322) reliées chacune avec l'une des parties superficielles cousues (110) et l'une des parties de support cousues (210) respectivement, les parties intermédiaires séquentielles (310, 312, 320, 322) étant uniquement composées de fils de chaîne intermédiaires,
**caractérisé en ce que**
la couche intermédiaire (300) comporte une structure multicouche, dans laquelle plusieurs couches de tissu sont séparées l'une de l'autre, où chaque partie intermédiaire (310, 312; 320, 322) forme une première couche de tissu et une seconde couche de tissu séparées.

2. Tissu 3D multicouche selon la revendication 1, où les plusieurs couches de tissu sont composées de premières parties intermédiaires (310, 312) et de secondes parties intermédiaires (320, 322) ; et les parties intermédiaires séquentielles (310, 312, 320, 322) sont reliées aux parties superficielles cousues (110) et aux parties support cousues (210) en alternant de manière répétitive, où les fils de chaîne intermédiaires qui relient les parties superficielles cousues (110) et les parties support cousues (210) et qui sont tissés sans entrelacement avec des fils de trame et qui ne composent pas les parties intermédiaires (310, 312, 320, 322) sont coupés.

3. Tissu 3D multicouche selon la revendication 1, où les plusieurs couches de tissu sont composées de premières parties intermédiaires (310, 312) et de secondes parties intermédiaires (320, 322) ; et les parties intermédiaires séquentielles sont reliées aux parties superficielles cousues (110) et aux parties support cousues (210) en alternant de manière répétitive, où les fils de chaîne intermédiaires qui relient les parties superficielles cousues (110) et les parties support non cousues (220) et qui ne composent pas les parties intermédiaires (310, 312, 320, 322) sont retirés.

4. Tissu 3D multicouche selon la revendication 1, où les parties superficielles cousues (110) sont composées des fils de chaîne superficiels et une partie des fils de chaîne intermédiaires; et les parties support cousues (210) sont composées des fils de chaîne support et d'une autre partie des fils de chaîne intermédiaires qui ne composent pas les parties superficielles cousues (110) ; et les parties intermédiaires séquentielles (310, 312, 320, 322) sont reliées aux parties superficielles cousues (110) et aux parties support cousues (210) en alternant de manière répétitive, où les fils de chaîne de liaison (313, 315) de la couche intermédiaire (300) qui reliaient respectivement les parties superficielles cousues (110) et les parties support cousues (210) sont coupés.

5. Tissu 3D multicouche selon la revendication 1, où les plusieurs couches de tissu sont composées de premières parties intermédiaires (310, 312) et de secondes parties intermédiaires (320, 322) et la couche superficielle (100) et la couche support (200) sont composées de leurs parties cousues respectives (110, 210), où les parties superficielles non cousues (120) et les parties support non cousues (220) sont en contact avec la couche intermédiaire (300), la couche superficielle (100) et la couche support (200) sont formées d'au moins deux fils de chaîne et les première et seconde parties intermédiaires (310, 312, 320, 322) sont composées d'un nombre pair d'au moins quatre fils de chaîne, les parties superficielles non cousues (120) et les parties support non cousues (220) sont formées par au moins deux fils de chaîne, des première et troisième parties superficielle cousues (111, 115) sont formées par des fils de chaîne des parties superficielles non cousues (120) et des fils de chaîne des premières parties intermédiaires (310, 312) et les deuxièmes parties superficielles cousues (113) sont formées par des fils de chaîne des parties superficielles non cousues (120) et des fils de chaîne des deuxièmes parties intermédiaires (320, 322), des première et troisième parties support cousues (211, 215) sont formées par les fils de chaîne des parties support non cousues (220) et les fils de chaîne des deuxièmes parties intermédiaires (320, 322) et les deuxièmes parties support cousues (213) sont formées par les fils de chaîne des parties support non cousues (220) et les fils de chaîne des premières parties intermédiaires (310, 312), les première et seconde parties intermédiaires (310, 312, 320, 322) sont formées par au moins deux fils de chaîne pour séparer les plusieurs couches de tissu, où les fils de chaîne de liaison de la couche intermédiaire (300) sont coupés.

6. Tissu 3D multicouche selon la revendication 1, où lorsque des fils de chaîne superficiels sont des premier et second fils de chaîne (1, 2), des fils de chaîne support sont des troisième et quatrième fils de chaîne (3, 4), des premiers fils de chaîne intermédiaires sont des cinquième, sixième, septième et huitième fils de chaîne (5, 6, 7, 8) et des seconds fils de chaîne intermédiaires sont des neuvième, dixième, onzième et douzième fils de chaîne (9, 10, 11, 12), comme indiqué par les numéros de harnais, les parties superficielles non cousues (120) et les parties support non cousues (220) sont essentiellement composées respectivement des premier et second fils de chaîne (1, 2) et des troisième et quatrième fils de chaîne (3, 4), les première et troisième parties superficielles (111, 115) de la couche superficielle (100) sont composées des premier, second, cinquième, sixième, septième et huitième fils de chaîne (1, 2, 5, 6, 7, 8) et la seconde partie superficielle cousue (113) est composée des premier, deuxième, neuvième, dixième, onzième et douzième fils de chaîne (1, 2, 9, 10, 11, 12), les première et troisième parties support cousues (211, 215) de la couche support (200) sont composées des troisième, quatrième, neuvième, dixième, onzième et douzième fils de chaîne (3, 4, 9, 10, 11, 12), la seconde partie support cousue (213) est composée des troisième, quatrième, cinquième, sixième, septième et huitième fils de chaîne (3, 4, 5, 6, 7, 8) et les premières parties intermédiaires (310, 312) forment une couche de tissu en utilisant les cinquième et sixième fils de chaîne (5, 6) et l'autre couche de tissu en utilisant les septième et huitième fils de chaîne (7, 8) pour les séparer l'une de l'autre, et les secondes parties intermédiaires 320, 322 forment une couche de tissu en utilisant les neuvième et dixième fils de chaîne (9, 10) et l'autre couche de tissu en utilisant les onzième et douzième fils de chaîne (11, 12) pour les séparer l'une de l'autre.

7. Tissu 3D multicouche selon la revendication 1, où les plusieurs couches de tissu sont composées de premières parties intermédiaires (310, 312) et de secondes parties intermédiaires (320, 322) et la couche superficielle (100) et la couche support (200) sont composées de leurs parties cousues respectives (110, 210), où les parties superficielles non cousues (120) et les parties support non cousues (220) sont en contact avec la couche intermédiaire (300) ; la couche superficielle (100) et la couche support (200) sont formées par au moins deux fils de chaîne et les première et seconde parties intermédiaires (310, 312, 320, 322) sont composées d'un nombre pair d'au moins quatre fils de chaîne, les parties superficielles non cousues (120) sont formées par au moins deux fils de chaîne, les première et seconde parties intermédiaires (310, 312, 320, 322) sont formées par au moins deux fils de chaîne pour séparer les plusieurs couches de tissu, des première et seconde parties support (211, 215) sont formées par des fils de chaîne des parties support non cousues (220) et des fils de chaîne des secondes parties intermédiaire (320, 322) et les secondes parties support cousues (213) sont formées de fils de chaîne des parties support non cousues et de fils de chaîne des premières parties intermédiaires (310, 312), la partie support non cousue (220) jusqu'à la première partie support cousue (211) et la partie cousue sont composées de fils de chaîne de la couche support (200) et de fils de chaîne des secondes parties intermédiaires (320, 322), la partie support non cousue (220) jusqu'à la seconde partie support cousue (213) et la partie cousue sont composées de fils de chaîne de la couche support (200) et de fils de chaîne des premières parties intermédiaires (310, 312), la partie support non cousue (220) jusqu'à la troisième partie support cousue (215) et la partie cousue sont composées de fils de chaîne de la couche support (200) et de fils de chaîne des secondes parties intermédiaires (320, 322), l'agencement précité étant séquentiellement répété, où les fils de chaîne des première et seconde parties intermédiaires (310, 312, 320, 322) reliant les parties superficielles cousues (110) et les parties support non cousues (220) et ne composant pas les parties intermédiaires (310, 312, 320, 322) sont retirés.

8. Tissu 3D multicouche selon la revendication 7, où lorsque des fils de chaîne superficiels sont des premier et second fils de chaîne (1, 2), des fils de chaîne support sont des troisième et quatrième fils de chaîne (3, 4), des premiers fils de chaîne intermédiaires sont des cinquième, sixième, septième et huitième fils de chaîne (5, 6, 7, 8) et des seconds fils de chaîne intermédiaires sont des neuvième, dixième, onzième et douzième fils de chaîne (9, 10, 11, 12), comme indiqué par les numéros de harnais, les parties superficielles non cousues (120) sont essentiellement composées respectivement des premier et second fils de chaîne (1, 2), les premières parties intermédiaires (310, 312) forment une couche de tissu à partir des cinquième et sixième fils de chaîne (5, 6) et l'autre couche de tissu à partir des septième et huitième fils de chaîne (7, 8) pour les séparer l'une de l'autre, et les secondes parties intermédiaires (320, 322) forment une couche de tissu à partir des neuvième et dixième fils de chaîne (9, 10) et l'autre couche de tissu à partir des onzième et douzième fils de chaîne (11, 12) pour les séparer l'une de l'autre, les première et troisième parties superficielles cousues (111, 115) de la couche superficielle (100) sont composées des premier, second, cinquième, sixième, septième et huitième fils de chaîne (1, 2, 5, 6, 7, 8) et la seconde partie superficielle cousue (113) est composée des premier, second, neuvième, dixième, onzième et douzième fils de chaîne (1, 2, 9, 10, 11, 12), les première et troisième parties support cousues (211, 215) de la couche support (200) sont composées des troisième, quatrième, neuvième, dixième, onzième et douzième fils de chaîne (3, 4, 9, 10, 11, 12), la seconde partie support cousue (213) est composée des troisième, quatrième, cinquième, sixième, septième et huitième fils de chaîne (3, 4, 5, 6, 7, 8), la partie support non cousue (220) jusqu'à la première partie support cousue (211) et la partie cousue sont composées des troisième, quatrième, neuvième, dixième, onzième et douzième fils de chaîne (3, 4, 9, 10, 11, 12), la partie support non cousue (220) jusqu'à la seconde partie support cousue (213) et la partie cousue sont composées des des troisième, quatrième, cinquième, sixième, septième et huitième fils de chaîne (3, 4, 5, 6, 7, 8), la partie support non cousue (220) jusqu'à la troisième partie support cousue (215) et la partie cousue sont composées des troisième, quatrième, neuvième, dixième, onzième et douzième fils de chaîne (3, 4, 9, 10, 11, 12), l'agencement précité étant répété séquentiellement.

9. Tissu 3D multicouche selon la revendication 1, où la couche superficielle (100) et la couche support (200) sont composées respectivement de leurs parties cousues respectives (110, 210), où les parties superficielles non cousues (120) et les parties support non cousues (220) sont en contact avec la couche intermédiaire (300), la couche superficielle (100) et la couche support (200) sont composées d'au moins deux fils de chaîne et les parties intermédiaires (310, 312, 320, 322) sont composées d'un nombre pair d'au moins quatre fils de chaîne, les parties superficielles non cousues (120) et les parties support non cousues (220) sont formées par au moins deux fils de chaîne, les parties intermédiaires (310, 312, 320, 322) sont formées par au moins deux fils de chaîne pour séparer les plusieurs couches de tissu, les parties superficielles cousues (110) sont composées de fils de chaîne superficiels et d'une partie des fils de chaîne des couches de tissu, les parties support cousues (210) sont composées de fils de chaîne support et d'une autre partie des fils de chaîne des couches de tissu qui ne composent pas les parties superficielles cousues (110), où des fils de chaîne de liaison (313, 315) qui reliaient respectivement les parties superficielles cousues (110) et les parties support cousues (210) sont coupés.

10. Tissu 3D multicouche selon la revendication 9, où lorsque des fils de chaîne superficiels sont des premier et second fils de chaîne (1, 2), des fils de chaîne support sont des troisième et quatrième fils de chaîne (3, 4), des fils de chaîne intermédiaires sont des cinquième, sixième, septième et huitième fils de chaîne (5, 6, 7, 8), comme indiqué par les numéros de harnais, les parties superficielles non cousues (120) sont essentiellement composées des premier et second fils de chaîne (1, 2) et les parties support non cousues (220) sont essentiellement composées des troisième et quatrième fils de chaîne (3, 4), les parties intermédiaires (310, 312, 320, 322) forment une couche de tissu à partir des cinquième et sixième fils de chaîne (5, 6) et l'autre couche de tissu à partir des septième et huitième fils de chaîne (7, 8) pour les séparer l'une de l'autre, les parties superficielles cousues (110) sont essentiellement composées des premier, second, sixième et huitième fils de chaîne (1, 2, 6, 8), les parties support cousues (210) sont essentiellement composées des troisième, quatrième, cinquième et septième fils de chaîne (3, 4, 5, 7).

11. Tissu 3D multicouche selon l'une quelconque des revendications 1 à 10, où le fil de chaîne et/ou le fil de trame est tissé à partir d'une fibre à bas point de fusion telle qu'une fibre composite thermofusible ayant un ingrédient à bas point de fusion et un ingrédient à haut point de fusion, où l'ingrédient à bas point de fusion forme en continu au moins une partie de la surface de la fibre dans la direction de la fibre, a une température de transition vitreuse de plus de 60°C et est composé d'un mélange d'1 à 20% en poids de polyolèfine et de 80 à 99 % en poids d'un copolyester ayant 50 à 70 %mol d'unités de polytéréphtalate d'éthylène.

12. Tissu 3D multicouche selon la revendication 11, où la fibre à bas point de fusion est une fibre grise dont le point de fusion est intentionnellement abaissé de sorte que sa surface puisse être fondue avec précision par traitement thermique à des températures d'environ 120°C à 190°C.

13. Tissu 3D multicouche selon l'une quelconque des revendications 1 à 10, où le fil de chaîne et/ou le fil de trame est une fibre grise, dans laquelle sont mélangées une fibre à bas point de fusion, telle qu'une fibre composite thermofusible ayant un ingrédient à bas point de fusion et un ingrédient à haut point de fusion, où l'ingrédient à bas point de fusion forme en continu au moins une partie de la surface de la fibre dans la direction de la fibre, a une température de transition vitreuse de plus de 60°C et est composé d'un mélange d'1 à 20% en poids de polyolèfine et de 80 à 99 % en poids d'un copolyester ayant 50 à 70 %mol d'unités de polytéréphtalate d'éthylène, et une fibre ignifugée ou bien une fibre composite ayant des parties à bas point de fusion et des parties ignifugées.

14. Tissu 3D multicouche selon la revendication 12, où le tissu est en outre traité thermiquement pour obtenir une stabilité de forme améliorée et une rigidité renforcée.

15. Tissu 3D multicouche selon l'une quelconque des revendications 1 à 10, où la couche superficielle (100) et la couche support (200) sont formées par tissage de manière à ce qu'elles aient une structure en mailles.

16. Tissu 3D multicouche selon l'une quelconque des revendications 1 à 10, où la couche intermédiaire (300) est plus dense que la couche superficielle (100) et la couche support (200).

17. Etoffe utilisant le tissu selon l'une quelconque des revendications 1 à 10.

18. Objet utilisant le tissu selon l'une quelconque des revendications 1 à 10.

19. Store utilisant le tissu selon l'une quelconque des revendications 1 à 10.
